

## UNITED STATES PATENT OFFICE

2,359,407

## PROTECTION OF METAL SURFACES FROM CORROSION

Ralph Forder Denington, Slough, England, assignor to Imperial Chemical Industries Limited, a corporation of Great Britain

No Drawing. Application February 6, 1942, Serial No. 429,806. In Great Britain March 31, 1941

7 Claims. (Cl. 148—6)

This invention relates to the protection of surfaces of metals against rusting or corrosion and to compositions suitable therefor. The invention relates particularly to the temporary protection of iron and steel against rusting during transit or storage, and during erection prior to painting.

It is well known that surfaces of ferrous metals may be prevented from corrosion or rusting by applying thereto a temporary coating of a waterproof material. These coatings may consist of clear lacquers or non-volatile oils, fats or greases, non-volatile in the sense that they can be applied to metal surfaces and do not evaporate under normal conditions of storage or transport. Mineral oil affords protection for a limited time only while in the case of thick greases such as lanoline a relatively deep layer is necessary to give appreciable protection.

We have now found that  $\beta$ -diketones have the property of reacting with iron compounds and remaining organophilic, and that when a small proportion of such a compound is applied to a metal surface, a protective layer is formed. Thus, if a proportion of such a compound is incorporated into a waterproofing material capable of being used as a temporary rust preventative, there results a composition of greatly enhanced value.

According to the present invention, therefore, surfaces of metals are protected against corrosion or rusting by application to the said surfaces of a composition consisting of or containing a  $\beta$ -diketone. The  $\beta$ -diketone may be applied as such or dissolved in a volatile organic solvent, and a surface so treated can subsequently be painted or lacquered without removing the protective film of the  $\beta$ -diketone. Alternatively the  $\beta$ -diketone can be applied, together with a waterproofing material of the kind customarily known or used in the art. For example the  $\beta$ -diketone may be dissolved in a clear lacquer or dispersed in a non-volatile oil, grease or fat, for example lanoline, or a mixture of these substances, or dispersed or dissolved in a solution of the oil, fat or grease in a volatile solvent.

The  $\beta$ -diketones used in accordance with the present invention have the general formula  $R-CO-CH_2-CO-R'$ , where  $R$  and  $R'$  can be alkyl or aryl or aralkyl groups, and may be similar or dissimilar. Examples of such compounds are undecylenyl acetone, oenanthyl acetone, caproyl acetone, capryl acetone, caprylyl

acetone, oleyl acetone, pelargonyl acetone, phenyl acetyl acetone and undecylenyl acetophenone.

The invention is illustrated by but not limited to the following examples.

Example 1

2 per cent of undecylenyl acetone was dissolved in toluol and poured on to a part of the surface of a steel panel exposed in the open air. It was found that corrosion of the steel commenced after 24 hours except on the area covered by the undecylenic  $\beta$ -diketone. This area showed no rust for 14 days.

Example 2

15 5 per cent of undecylenyl acetone was dissolved in thick gear oil and spread on a bright steel water-cooled surface. Under conditions of varying humidity, temperatures and condensation during a period of nine months no signs of corrosion were observed. Similar surfaces treated with gear oil alone showed spots of rust after one month.

Example 3

20 25 A composition comprising 20 parts by weight of lanoline with 2 parts by weight of undecylenyl acetone and 78 parts of petroleum distillate of boiling point within the range of 160° C. to 180° C. was applied to a clean mild steel surface exposed to weather. After ten weeks the film was removed with heavy naphtha, when it was found that the metal was bright and corrosion-free. By contrast a clean mild steel surface treated with a solution of lanoline in petroleum distillate showed appreciable corrosion.

Example 4

25 40 A composition comprising 20 parts by weight of lanoline, 2 parts by weight of undecylenyl acetone and 78 parts by weight white spirit when applied to clean mild steel and the solvent allowed to evaporate gave considerably greater protection than that obtained by the use of a lanoline solution alone.

Example 5

|                    | Parts by weight |
|--------------------|-----------------|
| Chlorinated rubber | 25              |
| Oleyl acetone      | 5               |
| Heavy naphtha      | 45              |
| Toluol             | 20              |
| Benzol             | 5               |

50 The chlorinated rubber was dissolved in the other components by stirring. The resulting composition was applied by brush to a steel girder which

was left exposed to the weather for a period of five months. On then removing the film by application of heavy naphtha the metal surface was found to be quite free from corrosion.

I claim:

1. A method of protecting metal surfaces against corrosion by exposure to the atmosphere which comprises applying to said surfaces a composition comprising a  $\beta$ -diketone.

2. A method of protecting metal surfaces against corrosion by exposure to the atmosphere which comprises applying to said surfaces a composition comprising a  $\beta$ -diketone and a volatile organic solvent.

3. A method of protecting metal surfaces against corrosion by exposure to the atmosphere which comprises applying to said surfaces a composition comprising a  $\beta$ -diketone and a material selected from the group consisting of non-volatile oils, fats, greases, mixtures of said materials, and solutions of said materials.

4. A method of protecting metal surfaces against corrosion by exposure to the atmosphere which comprises applying to said surfaces a composition comprising undecylenyl acetone.

5. A method of protecting metal surfaces against corrosion by exposure to the atmosphere which comprises applying to said surfaces a composition comprising oleyl acetone.

6. A method of protecting metal surfaces against corrosion by exposure to the atmosphere which comprises applying to said surfaces a composition comprising lauryl acetone.

7. A composition for the protection of metal surfaces against corrosion by exposure to the atmosphere which comprises oleyl acetone and a material selected from the group consisting of non-volatile oils, fats, greases, mixtures of said materials, and solutions of said materials.

RALPH FORDER DENINGTON.